

Jan. 8, 1929.

1,698,486

G. YUNGBLUT

PROCESS OF MAKING METALLIC SHEETS BY ELECTROPLATING

Filed Sept. 19, 1927



*Gibson Yungblut*  
INVENTOR.

*Allen & Allen*

ATTORNEYS.

Patented Jan. 8, 1929.

1,698,486

# UNITED STATES PATENT OFFICE.

GIBSON YUNGBLUT, OF DAYTON, KENTUCKY, ASSIGNOR TO THE RICHARDSON COMPANY, OF LOCKLAND, OHIO, A CORPORATION OF OHIO.

## PROCESS OF MAKING METALLIC SHEETS BY ELECTROPLATING.

Application filed September 19, 1927. Serial No. 220,356.

My invention relates to the production of metallic sheets or other articles by electrodeposition of metal upon a base plate from which the deposited metal is subsequently freed by an electrolytic differential solution stripping step. In a separate application filed by the present applicant and John R. Cain, such a process is described, in which for example, a double thickness plate of copper is placed in an electrolytic cell and has deposited upon it a double thickness plate of iron. This composite plate is then rolled so as to double its length and halve its thickness, is cut into two parts, and both parts are placed in a suitable stripping cell. The action of this cell when iron sheets are desired as a finished product will be controlled so that the copper will be entirely dissolved from one of the iron sheets and built up upon the copper face of the corresponding copper-iron sheet.

The bare iron sheet is then, so far as this process is concerned, a finished product. The copper-iron plate, consisting of a double thickness of copper and a single thickness of iron, is then returned to the iron plating bath, and the process is repeated cyclically.

It is the object of this invention to permit the production of sheets of electrolytic metal upon base plates from which they are subsequently removed without having been rolled at all. My processes although useful in the production of other kinds of sheets, is thus particularly adapted to the making of extremely thin metallic bodies, foils of iron or iron alloys for transformer use, and especially foils of the precious metals.

It is another object of my invention to provide in such a process means continuously to regenerate the base plates.

It is another object of my invention to provide means whereby the base plate surface will always be clean, bright and rolled when it is plated upon. My process does away with the thickening of an electrodeposit previously formed and previously worked in connection with a base plate, so that my electrolytically deposited sheets will always be formed with one face freshly deposited against a freshly polished surface.

It is another object of my invention to do away with any necessary relationship between the hardening and thickening of the base plate and the hardening and thickening of the electrodeposited sheet thereon, so as to

permit the depositing of extremely thin foils upon a base plate so thick as to be conveniently handled, or the depositing of thick sheets upon base plate so thin as to minimize the time and current consumption of the stripping process.

It is another object of my invention to form an electrodeposited finished product which, because it need not be rolled, need not be annealed or otherwise treated. Metals and particularly iron when electrodeposited have certain crystalline structures and electric and magnetic properties which are altered by subsequent treatments and may not thereafter be restored.

It is another object of my invention to provide, in a system involving the regeneration of base plates, means of compensating for the loss of metal in trimming after the rolling operation.

Other objects will be apparent to those skilled in the art upon reading these specifications.

I accomplish my objects by that certain series of steps which will hereinafter be specifically pointed out in a typical example and the novelty inherent in which will be set forth in the claims that follow.

### In the drawings:

The figure is a diagram in which the sheets and base plates are represented in side elevation and which shows the various named steps of my process.

Since my invention consists in the novel combination of steps, no attempt is made in the drawings to illustrate other than diagrammatically various rolling and electrolytic processes which are within the knowledge of one skilled in the art to perform.

My process involves the use of two base plates, or series of base plates, of one metal M, which I have indicated in the figure as M-1 and M-2. The finished sheets which I desire are of a different metal indicated as N.

The process consists, briefly, in placing a base plate M-1 in an electrolytic bath A in which is an electrolyte B comprising a solution of the salt of the metal N. A suitable anode C is placed in the cell and through the action of a source of electrical energy, not shown, connected both to the anode and the cathode of the electrolytic couple, an electrodeposit of the metal N is formed upon the cathodic base plate M-1. The product of

this operation, designated as M-1-N, is transferred to an electrolytic stripping cell D in which the base plate M-1 is dissolved, leaving as an end product the desired metallic plate N.

In the electrolytic stripping cell D the electrolyte is a solution of a salt of a metal M which will attack under electrolytic conditions and dissolve the metal M from the composite anode but will have no effect upon the metal N.

I use as a cathode in this cell a second base plate of the metal M which I have indicated as M-2. The metal M-1 dissolved from the anode will be deposited on this cathode and the resulting cathode at the end of the stripping operation is a plate approximately double the thickness of the original base plate. I have indicated this as M-1-M-2. After washing, this cathode is passed one or more times through suitable rolls with intervening annealing operations if necessary, so that its thickness is halved and its length doubled, whereupon it is cut into two parts.

It will be obvious that the result of this process is to regenerate the plates M-1 and M-2. M-1 is transferred back to the electrolytic cell A and M-2 to the electrolytic stripping cell D.

It will be seen that I have formed my finished product N by the simple operation of forming it electrolytically upon a cathode blank and then freeing it from said blank by an electrolytic differential solution step. It has not been rolled, annealed or otherwise treated, and the advantages of this process in forming foils from metallic deposits so thin that they cannot be worked or rolled will be immediately apparent.

In the commercial operation of my process M-1 and M-2 will represent series of blanks rather than single ones, and the number of couples in the series A and D, if the couples are connected in parallel, may be increased as much as desired, or the number of cells increased if the couples are connected in series.

The rolling operation will necessitate trimming off the edges and it will be seen that since the blanks M-1 and M-2 are already

trimmed and of proper thickness, some means must be taken for compensating for the trim, or in other words, for increasing the amount of metal in the composite M-1-M-2. Another way of stating this is to say that the composite M-1-M-2 before rolling must contain a weight of metal equivalent to M-1 plus M-2 plus the average or necessary trim, if the thickness of the plates M-1 and M-2 is not continuously to diminish.

I compensate for this trim by placing in the stripping cell a supplementary anode M-3 connected to a source of current (which will also be connected to the cathode M-2) of such value as to deposit upon M-2 a weight of metal equivalent to the calculated neces-

sary trim during the time required by the stripping of M-1 from the finished plate N. Thus the cathode taken from the stripping cell at the end of the stripping operation will consist of M-1 plus M-2 plus some metal from the supplementary anode. If the weight of metal in M-1 and M-2 is indicated as X and the weight of the calculated trim as Y, the weight of the composite cathode from the stripping bath may be expressed as 2X plus Y. After rolling, trimming and cutting, therefore, M-1 and M-2 would be regenerated and there would be left over an amount of trim equivalent to the weight of metal deposited from the supplementary anode. In the commercial operation this trim will be remelted and cast into supplementary anodes M-3, or may be used in a basket or some other device which will make remelting unnecessary.

I will now describe the operation of my invention in a typical example, that is to say, the formation of very thin iron sheets on a base plate of copper. I start with a base plate of copper of any desired thickness, which may conveniently be .02". The thickness will be controlled by the operator in accordance with his convenience in handling the size of sheet to be produced, and it will be seen that in a process for the production of metallic bodies of comparative thinness, the size and shape of the cathode blank or plate will determine the size and shape of the finished electrodeposited article. Thus in the manufacture of thin electrolytic iron for electrical purposes, the cathode blank M may be stamped or cut into a certain configuration as, for example, the core of a transformer or armature. Resort may be had to shielding or other devices for preventing the electrodeposit of iron around the edges or upon the reverse side of the cathode blank, or the cathode blank may be treated with an insulating compound over the portions upon which no deposit is desired. In this manner two or more finished articles may be formed upon one cathode blank. This is of particular advantage where numerous small articles are desired.

I prefer to employ in the cell A for the manufacture of soft electrolytic iron the process outlined in the application of John R. Cain, filed March 8, 1927, Serial No. 173,794, and the anode described in John R. Cain's application filed March 8, 1927, Serial No. 173,793.

Electrical connection is made with a direct current low voltage dynamo or other source of electrical energy and iron is deposited upon the desired portions of the cathode blank to the thickness required in the finished product.

I then remove the cathode blank M-1 with its adhering deposit or deposits of iron and place it in a separate electrolytic cell

containing as an electrolyte a solution comprising cupric cyanide. The operation in this cell is set forth and claimed in the application of John R. Cain filed June 11, 1926, Serial No. 115,405. I use as a cathode the second copper blank M-2, which is also .02" in thickness and similar in all respects to the blank M-2. With a suitable source of current, I carry on a differential stripping of the copper from the composite blank M-1-N, placing in my cell supplementary anodes of cast copper M-3 connected to a supplementary source of current of such value as will deposit upon the cathode blank a weight of metal calculated to compensate for the trim. This will obviously vary with the size of the sheet to be produced and the character of the rolling operation.

In cases where I am producing more than one iron article upon a single copper cathode blank, I take care to see that each article is connected individually to the source of electrical energy. The reason for this is that as stripping action progresses, the copper plate may be dissolved unequally and if a part of it were detached and fell to the bottom of the tank so as to break its electrical connection with the positive side of the current source, stripping action on this piece would stop. This may be taken care of by supplementary connections or by leaving, through the insulation applied to the face of the plate M-1, paths permitting the deposition of iron and leading to the point at which current connection will be made.

Copper hardens rapidly upon working and I have found it, therefore, advantageous to anneal the copper cathode indicated in Figure 1 as M-1-M-2 after one or more passes through the cold rolls. I prefer to use for this annealing a bath of hydrocarbon oil heated to around 400° centigrade such as is described in the application of John R. Cain filed June 17, 1926, Serial No. 116,723. This annealing operation does not result in the formation of any scale or oxide, and after annealing, if the piece is to be returned to the rolls, it is only necessary to pass it through rubber rollers or some similar wiping device to remove the excess oil.

After the required reduction has been accomplished, however, and the rolled piece trimmed and cut apart into the regenerated plates M-1 and M-2, I remove the residual oily film with a solvent before returning the plates to the several cells, so that electrolytic action can take place unimpaired. A pickling step may be resorted to if desired, though I have not usually found this requisite. The trim from successive regeneration steps, I melt in a small furnace and cast into the supplementary anodes M-3.

While in a specific example I have described my process in connection with certain definite electrolytic steps, I desire it to be understood

that the invention is not limited to any specific metals or any specific electrolytic processes. For example, in the iron plating step, instead of using the sulphide of iron anodes described in the patent application referred to, I may use an electrolytic step involving the use of insoluble anodes and the consequent depletion of the metal content of the electrolyte, renewing my electrolyte in a leaching step. I may thus produce articles of any metal capable of being deposited on another metal from an electrolyte, and I may use as my starting blank any metal capable of being electrolytically stripped in an electrolytic differential solution step and redeposited in the same step upon a cathode.

Furthermore, while I have described my process as involving the use of sheets and as being a sheet-forming process, it is nevertheless applicable to the formation of other things besides sheets as, for example, in the manufacture of thin walled tubing. In such a process the blank M-1 would be a tube. Within this tube would be placed a central axial anode of the metal N, and the electrolyte B would be placed within the tube or caused to flow through it. The action of an electric current would deposit a tube of the metal M within the blank N to the required thickness. In the stripping cell D both the cathode and anode would preferably rotate and the metal M would be deposited upon the outside of the blank M-2. The resultant composite cathode M-1-M-2 would be a double-thickness tube which with suitable intervening annealings, would be passed through a tube-drawing die, its length doubled and its wall diameter halved, whereupon it would be cut apart into regenerated tubes M-1 and M-2. The trim or wastage in the tube-drawing step would be compensated for in the same fashion through the use of supplementary anodes M-3 and a supplementary source of current.

Having thus described my invention what I claim as new and desire to secure by Letters Patent is:

1. A process for forming electrolytic metal articles which consists in providing a cathode shaped like the article, but of another metal, plating it on one face with the desired metal and then stripping the cathode metal from the plated body in an electrolytic cell in which a like cathode is used and upon which the stripped metal is plated.

2. A process for forming electrolytic metal articles which consists in providing a cathode shaped like the article, but of another metal, plating it on one face with the desired metal and then stripping the cathode metal from the plated body in an electrolytic cell in which a like cathode is used and upon which the stripped metal is plated, and then reducing the thickness of the last noted cathode to

provide a new set of cathodes for both steps of the process.

3. A process for forming electrolytic metal articles which consists in providing a cathode shaped like the article, but of another metal, plating it on one face with the desired metal and then stripping the cathode metal from the plated body in an electrolytic cell in which a like cathode is used and upon which the stripped metal is plated, and then reducing the thickness of the last noted cathode to provide a new set of cathodes for both steps of the process, said cathodes being in the form of flat plates.
- 15 4. A process for forming electrolytic metal articles which consists in providing a cathode shaped like the article, but of another metal, plating it on one face with the desired metal and then stripping the cathode metal from the plated body in an electrolytic cell in which a like cathode is used and upon which the stripped metal is plated, and then reducing the thickness of the last noted cathode to provide a new set of cathodes for both steps

of the process, there being additional cathode 25 metal used as anodic material in said stripping cell, so as to plate the cathode therein up to sufficient thickness to allow for scrap in the step of reduction of thickness.

5. A process for forming electrolytic iron 20 articles which consists in providing a copper cathode shaped like the desired article, plating it with iron on one face, and then stripping the copper from the iron in an electrolytic cell in which a copper cathode is provided 35 and onto which the stripped copper is plated.

6. A process for forming electrolytic iron articles which consists in providing a copper cathode shaped like the desired article, plating it with iron on one face, and then stripping the copper from the iron in an electrolytic cell in which a copper cathode is provided 40 and onto which the stripped copper is placed, then rolling the newly plated cathode 45 to extend its length thus providing new cathodes for a further series of like steps.

GIBSON YUNGBLUT.